

July 18, 1939.

J. M. MICHEL

2,166,365

TREATMENT OF METALS

Filed Aug. 25, 1938

*Fig. 1.*



*Fig. 2.*



*Inventor*

Josef Martin Michel

By His Attorneys *Hutz and Joslin*

## UNITED STATES PATENT OFFICE

2,166,365

## TREATMENT OF METALS

Josef Martin Michel, Bitterfeld, Germany, assignor to I. G. Farbenindustrie Aktiengesellschaft, Frankfort-on-the-Main, Germany

Application August 25, 1938, Serial No. 226,738  
In Germany August 28, 1935.

13 Claims. (Cl. 148—13.1)

This invention relates to improvements in the treatment of metals and is a continuation in part of my application bearing Serial Number 95,015 and filed in the United States Patent Office on 5 August 8, 1936, bearing the title "Heat-treatment of magnesium alloys", and also of my application bearing Serial Number 143,908 and filed in the United States Patent Office on May 21, 1937, bearing the title "Process of improving workpieces 10 made from metals of the iron group and their alloys".

In the United States Patent specification 2,036,- 563 entitled "Heat-treatment of magnesium alloys", there is described and claimed a process for 15 the heat-treatment of light metal alloys containing magnesium, which comprises submerging the alloys in a bath substantially consisting of molten anhydrous sodium bichromate or potassium bichromate, or mixtures thereof, the preferred portion 20 in such mixtures being one part of potassium dichromate to three parts of sodium dichromate.

In using such baths for the heat-treatment, at 25 temperatures above 400° C., of workpieces of for example, aluminium-base alloys containing magnesium, or of metals of the iron group and their alloys, it is found, especially when the baths are kept in use over prolonged periods, that decomposition phenomena occur which lead to the deposition 30 of sludgy products which have been shown by investigation to consist chiefly of chromic oxide, whilst the viscosity of the saline bath gradually increases. This decomposition further results in a progressive change in the composition 35 of the bath and also in some cases in the setting up of an injurious reaction with the surface of the workpieces under treatment. This is particularly the case, when the fused saline baths contain, or consist of fused alkali metal dichromates, because 40 increasing temperatures are accompanied by a progressive decomposition of the dichromates, with the formation of monochromate and chromium oxide, in accordance with the equation:



45 where Me denotes either sodium or potassium, or a mixture of both cations. This reaction continues until a certain ratio between dichromate and monochromate has been reached which represents 50 a state of equilibrium which varies with the temperature, in the sense that, for a bath of given composition, there is a well-defined partial oxygen pressure corresponding to each temperature. This theory regarding the course of the decomposition reaction has been confirmed by the fact

that the oxidation value of a melt composed of sodium dichromate and/or potassium dichromate asymptotically decreases to a certain definite value when the melt is left for some considerable time at a constant temperature above 400° C. 5

It has now been ascertained that this decomposition of potassium dichromate is counteracted, if the fused saline baths also contain an amount of potassium monochromate at least corresponding to the constant oxidation value of the melt (in 10 the absence of monochromate) at the working temperature employed. The monochromate may be added as such, to the bath, or the desired ratio of dichromate to monochromate can be obtained by the addition of corresponding quantities of 15 salts such as potassium nitrate which are capable of transforming dichromate into monochromate. The potassium salts may be partially, or wholly, replaced by the corresponding sodium salts. The accompanying drawing contains two graphs, 20 which have been drafted on the basis of experiments. These graphs make it possible, in a simple manner, for a given application temperature of a saline bath to ascertain the exact ratio between sodium bichromate, potassium bichromate, and sodium monochromate, potassium monochromate, respectively, to be used in accordance with the present invention. In view of the circumstance, however, that in practical working 25 the prescribed temperature of the bath is occasionally exceeded, it is advisable to employ, in the melt, a slightly larger amount of monochromate than would be required to just compensate for the ascertained constant oxidation value of the monochromate-free melt, at the temperature concerned. 30

For a complete understanding of my invention, reference is made to the accompanying drawing in which, Fig. I is a graph in which oxidation values are plotted against temperatures and Fig. 40 II is a graph in which oxidation values are plotted against the equilibrium ratios of various mixtures of mono chromates and dichromates.

In Fig. I the oxidation values, calculated on the basis of chromic acid titre=cubic centimetres of 45 1/10 normal solution of  $\text{Na}_2\text{S}_2\text{O}_3$ /1 grm. (ordinates), are plotted against temperatures (abscissae). Fig. I thus enables one to ascertain the oxidation value of a bath for a given temperature simply by following the temperature ordinate until it intersects the curve, and from that point running along the corresponding abscissa, until the latter strikes the ordinate axis, from which the oxidation value corresponding to the given temperature is read. 50

In Fig. II the equilibrium ratios between baths consisting of

5       $\text{Na}_2\text{CrO}_4$  and  $\text{Na}_2\text{Cr}_2\text{O}_7$   
        $\text{Na}_2\text{CrO}_4$  and  $\text{K}_2\text{Cr}_2\text{O}_7$   
        $\text{K}_2\text{CrO}_4$  and  $\text{Na}_2\text{Cr}_2\text{O}_7$   
        $\text{K}_2\text{CrO}_4$  and  $\text{K}_2\text{Cr}_2\text{O}_7$

10     are plotted against the oxidation values as defined in connection with the graph of Fig. I, the abscissa values running from left to right for the bichromates, and from right to left for the monochromates. Taking therefore the oxidation value ascertained for a bath of a given temperature from Fig. I, it is only necessary to follow the parallel to the abscissa axis through the ordinate corresponding to the given oxidation value, and ascertain the abscissae of the points at which that parallel intersects the equilibrium lines, representing the respective binary systems.

15     Taking for instance a temperature of 500° C., Fig. I gives an oxidation value of 207, and this latter when followed up in Fig. II, shows that both a melt consisting of about 58%  $\text{Na}_2\text{Cr}_2\text{O}_7$  and 42%  $\text{Na}_2\text{CrO}_4$ , and also a melt consisting of about 25%  $\text{Na}_2\text{Cr}_2\text{O}_7$  and 24%  $\text{K}_2\text{CrO}_4$ , will be in equilibrium at that temperature.

20     For an annealing temperature of 650° C. baths of the following composition, for example, are suitable:

- 25     (a) 82 parts of  $\text{K}_2\text{Cr}_2\text{O}_7$  and 18 parts of  $\text{KNO}_3$   
       (b) 63 parts of  $\text{K}_2\text{Cr}_2\text{O}_7$  and 37 parts of  $\text{K}_2\text{CrO}_4$   
       (c) 42 parts of  $\text{Na}_2\text{Cr}_2\text{O}_7$  and 58 parts of  $\text{K}_2\text{CrO}_4$

30     The foregoing mixtures have an oxidation value of 185, which is thus about 6 points below the value corresponding to equilibrium at 650° C. so that increases of temperatures to about 700° C. for short periods can be permitted without appreciably altering the composition of the bath.

35     The content of monochromate thus required is, in the case of temperatures between 400° and 500° C. at least about 5%, but preferably slightly higher, for example from 7 to 10%. The effect of this proportion of monochromate in the dichromate baths is that decomposition phenomena, accompanied by the deposition of sludgy products, are prevented from occurring at temperatures above 400° C.

40     In the preparation of baths in accordance with the invention, the requisite amount of monochromate can be added, as such, to the dichromate bath, or the monochromate can be formed in the bath itself, by adding to the latter suitable amounts of substances, such as caustic alkalis, alkali peroxides, alkali nitrates, and also alkali carbonates, which are adapted to convert dichromate into monochromate in the melt.

45     The fused saline baths of the present invention exhibit the further advantage that corrosion of the bath containers such as is sometimes observed particularly in the case of iron vessels when using purely dichromate baths, is completely avoided.

50     The invention will now be illustrated with reference to the following comparative tests:

55     A mixture of 750 parts by weight of sodium dichromate and 250 parts by weight of potassium dichromate is fused in an iron vessel and then heated to 500° C. Test pieces of aluminium-magnesium alloys are then immersed in the melt. 60     After 24 hours, sludgy deposits already appear in the bath, increasing progressively as time goes on and finally rendering the melt viscous and unsuitable for practical use. The initial oxidation value of 220 cc. of n/10  $\text{Na}_2\text{S}_2\text{O}_3$  per 1 grm. 65     of the melt had fallen to 208 after 10 days. Analysis

70     of the sludge showed the presence of chromic oxide contaminated with 20% of ferric oxide, resulting from the action of the liberated oxygen on the walls of the vessel.

75     If, on the other hand, in accordance with the invention, there are added to the mixture of alkali dichromates fused in the foregoing manner, 30 parts by weight of potassium hydrate (90% concentration) corresponding to 23 parts by weight of  $\text{K}_2\text{O}$ , the oxidation value of 206.5, determined in the melt before use, remains unchanged after 3 weeks' service. No deposit is observed.

80     The same effect can be obtained by an addition of 21 parts by weight of caustic soda.

85     The same results are obtained by treating the saline mixture, prepared as above, with 50 parts by weight of potassium nitrate and employing the mixture at 500° C. The following oxidation values are obtained:

90     First day of test: Oxidation value 207.

95     Twentieth day of test: Oxidation value 207.

100     The bath functions without any decomposition.

105     The same effect is likewise obtained when the mixture of 750 parts of sodium dichromate and 250 parts of potassium dichromate is treated with 100 parts by weight of monochromate

110     (75  $\text{Na}_2\text{CrO}_4$ +25  $\text{K}_2\text{CrO}_4$ )

115     in which case the oxidation values are:

120     First day of test: 207.

125     Twentieth day of test: 206.

130     In this case also no appreciable deposit is observed.

135     It has been observed that the resistance to incidental and subsequent corrosion of workpieces made of numerous metals of the iron group, and of their alloys, is extensively diminished, or practically prevented altogether by the treatment with the fused saline baths according to the invention, as the following summary will show: .

140     Temperature of test: 500° C.

145     Duration of test: 11 days.

150     1. *Saline melt.*—750 grms. of  $\text{Na}_2\text{Cr}_2\text{O}_7$ +250 grms. of  $\text{K}_2\text{Cr}_2\text{O}_7$  (without added stabiliser).

| Material                 | Loss in weight in grammes per sq. metre per diem (representing incidental corrosion) | 45 |
|--------------------------|--------------------------------------------------------------------------------------|----|
| Iron.....                | 30 to 35                                                                             | 50 |
| Chrome-nickel steel..... | 7 to 8                                                                               |    |
| Nickel.....              | 6 to 7                                                                               |    |

160     2. *Saline melt.*—750 grms. of  $\text{Na}_2\text{Cr}_2\text{O}_7$ +250 grms. of  $\text{K}_2\text{Cr}_2\text{O}_7$ +10% of  $\text{K}_2\text{CrO}_4$  (according to the present invention),

| Material                 | Loss in weight in grammes per sq. metre per diem (representing incidental corrosion) | 60 |
|--------------------------|--------------------------------------------------------------------------------------|----|
| Iron.....                | 2 to 3                                                                               | 65 |
| Chrome-nickel steel..... | 0.7 to 0.8                                                                           |    |
| Nickel.....              | 0.6 to 0.7                                                                           |    |

65     This result is primarily attributable to the formation of protective layers on the surface of the materials in the stabilised baths. Thus, it was observed that, even in the case of an immersion of comparatively short duration, as is the rule for purposes of heat-treatment of metals of high melting point, such as nickel, iron, Monel metal and chrome-nickel steels of the most diverse com- 70

75

position, firmly adherent coatings of a colour ranging from dark brown to black, according to the duration of contact, are formed on the work-pieces. It has been found that, especially in the case of iron and its alloys, in addition to the good browning effect, such protective layers produce a particularly durable improvement of the surface, so that rusting on exposure to air is either substantially lessened, or even practically eliminated. Consequently, these coatings are especially suitable as a priming for the subsequent application of coloured lacquers and the like.

The following table shows the influence of a preliminary treatment at 500° C., with fused saline baths according to the invention over various periods on the subsequent corrosion resistance for various commercial metals, the extent of corrosion having been determined by direct measurement of the current strength in a 2% solution of sodium chloride (Tödt method). In each case, the reading was taken after immersion for 2 minutes.

| 25 | Material                                          | Immersion in bath, minutes | Corrosion in amperes per sq. cm. $\times 10^{-3}$ | Improvement, percent |
|----|---------------------------------------------------|----------------------------|---------------------------------------------------|----------------------|
|    | I. Iron:                                          |                            |                                                   |                      |
|    | (a) Untreated.....                                |                            | 8.5 to 9.5                                        | -----                |
| 30 | (b) Treated in accordance with the invention..... | 2                          | 6.3                                               | 30                   |
|    |                                                   | 5                          | 5.9                                               | 34.5                 |
|    |                                                   | 10                         | 5.3                                               | 41                   |
|    |                                                   | 20                         | 4.3                                               | 52                   |
|    |                                                   | 40                         | 4.7                                               | 48                   |
|    | II. Nickel:                                       |                            |                                                   |                      |
|    | (a) Untreated.....                                |                            | 1.0                                               | -----                |
| 35 | (b) Treated in accordance with the invention..... | 30                         | 0.6                                               | 40                   |
|    |                                                   | 60                         | 0.3                                               | 60                   |
|    |                                                   | 120                        | 0.3                                               | 60                   |
|    | III. Monel metal:                                 |                            |                                                   |                      |
|    | (a) Untreated.....                                |                            | 1.7                                               | -----                |
| 40 | (b) Treated in accordance with the invention..... | 10                         | 0.7                                               | 59                   |
|    |                                                   | 20                         | 0.3                                               | 82.5                 |

I claim:

1. A process for the heat-treatment of metals and alloys included in the group consisting of the metals of the iron group and their alloys, and light metal alloys containing magnesium, which comprises submerging said metals or alloys in a bath, substantially consisting of at least one molten anhydrous compound of the group consisting of sodium bichromate and potassium bichromate, and at least one compound of the group consisting of sodium monochromate and potassium monochromate, the content of monochromate being at least approximately corresponding to the equilibrium ratio between dichromate and monochromate at the temperature of the heat-treatment.
2. A process for the heat-treatment of metals and alloys included in the group consisting of the metals of the iron group and their alloys, and light metal alloys containing magnesium, which comprises submerging said metals or alloys in a bath substantially consisting of about three parts of anhydrous sodium bichromate and about one part of anhydrous potassium bichromate, and at least one compound of the group consisting of sodium monochromate and potassium monochromate, the content of monochromate being at least approximately corresponding to the equilibrium ratio between dichromate and monochromate at the temperature of the heat-treatment.
3. A process for the heat-treatment of light-metal alloys containing magnesium at tempera-

tures between 400° and 500° C., which comprises submerging said alloys in a bath, substantially consisting of at least one molten anhydrous compound of the group consisting of sodium bichromate and potassium bichromate, and at least about 5% by weight of an alkali monochromate.

4. A process for the heat-treatment of light-metal alloys containing magnesium at temperatures between 400° and 500° C., which comprises submerging said alloys in a bath, substantially consisting of at least one molten anhydrous compound of the group consisting of sodium bichromate and potassium bichromate and between about 7% and about 10% by weight of an alkali monochromate.

5. A molten saline bath for the heat-treatment of metals and alloys included in the group consisting of the metals of the iron group and their alloys, and light metal alloys containing magnesium, which bath substantially consists of at least one molten anhydrous compound of the group consisting of sodium bichromate and potassium bichromate, and at least one compound of the group consisting of sodium monochromate and potassium monochromate, the content of monochromate being at least approximately corresponding to the equilibrium ratio between dichromate and monochromate at the temperature at which the bath is to be used, and said bath being substantially free from sludge.

6. A molten saline bath for the heat-treatment of metals and alloys included in the group consisting of the metals of the iron group and their alloys, and light-metal alloys containing magnesium, which bath substantially consists of about three parts of anhydrous sodium bichromate and about one part of anhydrous potassium bichromate and at least one compound of the group consisting of sodium monochromate and potassium monochromate, the content of monochromate being at least approximately corresponding to the equilibrium ratio between dichromate and monochromate at the temperature at which the bath is to be used, and said bath being substantially free from sludge.

7. A molten saline bath for the heat-treatment of light-metal alloys containing magnesium at temperatures between 400° and 500° C., which bath substantially consists of at least one molten anhydrous compound of the group consisting of sodium bichromate and potassium bichromate, and at least about 5% by weight of an alkali monochromate, said bath being substantially free from sludge.

8. A molten saline bath for the heat-treatment of light-metal alloys containing magnesium at temperatures between 400° and 500° C., which bath substantially consists of at least one molten anhydrous compound of the group consisting of sodium bichromate and potassium bichromate, and between about 7% and about 10% by weight of an alkali monochromate, said bath being substantially free from sludge.

9. A molten saline bath for the heat-treatment of metals and alloys included in the group consisting of the metals of the iron group and their alloys, and light-metal alloys containing magnesium, substantially consisting of anhydrous dichromates and monochromates, in which the ratio of monochromate to dichromate at least corresponds to the equilibrium ratio between monochromate and dichromate at the temperature of the bath, and said bath being substantially free from sludge.

10. A method of preparing a bath of the kind

described for the heat-treatment of metals and alloys included in the group consisting of the metals of the iron group and their alloys, and light metal alloys containing magnesium, which comprises adding to a fused bath substantially consisting of alkali dichromates a substance adapted to convert dichromate into monochromate in proportion corresponding at least to the equilibrium ratio between monochromate and dichromate at the temperature at which the bath is to be used, and said bath being substantially free from sludge.

11. A method of preparing a bath of the kind described for the heat-treatment of metals and alloys included in the group consisting of the metals of the iron group and their alloys, and light metal alloys containing magnesium, which comprises adding to a fused bath substantially consisting of alkali dichromates a substance selected from the group consisting of the caustic alkalis, alkali metal peroxides, alkali metal nitrates, and alkali metal carbonates, in such proportion as to establish, by conversion of part of

such dichromates into monochromates, a ratio between monochromate and dichromate in said bath corresponding at least to the equilibrium ratio between monochromate and dichromate at the temperature at which the bath is to be used, and said bath being substantially free from sludge. 5

12. A process for the heat-treatment of metals of the iron group and their alloys at temperatures of about 650° C., which comprises submerging said metals or alloys in a fused bath, substantially consisting of about 42 parts by weight of sodium bichromate and about 58 parts of potassium monochromate. 10

13. A process for the heat-treatment of metals of the iron group and their alloys at temperatures of about 650 C., which comprises submerging said metals or alloys in a fused bath substantially consisting of about 63 parts by weight of sodium bichromate and about 37 parts of potassium monochromate. 15 20

JOSEF MARTIN MICHEL.